

## UNITED STATES PATENT OFFICE

2,328,431

## PROCESS FOR RENDERING TEXTILE MATERIALS WATER REPELLENT

Arnold Doser, Cologne, and Otto Bayer and Karl Hintzmann, Leverkusen I. G.-Werk, Germany, assignors, by mesne assignments, to General Aniline & Film Corporation, New York, N. Y., a corporation of Delaware

No Drawing. Application May 16, 1939, Serial No. 274,025. In Germany May 17, 1938

3 Claims. (Cl. 117—167)

The present invention relates to a process for rendering textile materials water-repellent with the aid of zirconium compounds and constitutes a further development of the processes described in our co-pending application Serial No. 221,452, filed July 26, 1938.

We have found that textile materials of various origin can be rendered excellently and permanently water-repellent by impregnating the materials with a water-repellent compound selected from the group consisting of paraffin, wax and fatty compounds, and with a zirconium compound, and thereupon treating the material in an aqueous neutral to alkaline bath, whereby the hydrophilic substances are removed therefrom as far as possible, and finally drying the material at elevated temperature.

In its most general aspect the present invention may be carried out with various kinds of zirconium compounds like, for instance, those compounds which give strongly acid aqueous solutions or dispersions like, for instance, zirconium oxychloride, zirconium oxynitrate and the water soluble or dispersible hydrolysates obtainable therefrom, moreover, zirconium sulfate, zirconium acetate, zirconium acetonitrile, zirconium formate, etc. The quantity of the zirconium compounds to be used in the present process depends somewhat on the desired degree of water-repellency, in a manner which is easily understood by those skilled in the art; the same holds true for the quantity of paraffins, waxes and/or fatty compounds to be used together with the zirconium compounds. Besides zirconium compounds, compounds of suitable other metals may be present, as for instance, soluble or dispersible compounds of aluminium, chromium, thorium, cerium, titanium or of the metal mixtures contained in monazite sand. A good effect is obtained already when less than 1% of the zirconium compound is brought on the textile material; if necessary, this quantity may also be increased. In any case, however, the quantities of zirconium compound necessary for producing the desired result are smaller than those which have been employed in known processes for leading silk fabrics.

Impregnating of the textile material with the water-repellent organic substances and with the zirconium compounds may be carried out at normal or elevated temperature, for instance, at 40–50° C. The water-repellent organic substances are preferably used in the form of aqueous emulsions which may be prepared with the aid of suitable emulsifying agents, for instance, with

the aid of soap or of non-soapy highly efficient synthetic emulsifiers like, for instance, condensation products of high molecular aliphatic compounds like oleyl alcohol with an excess ethylene oxide (see German specification No. 605,973), condensation products of colophony and phenols having been treated with an excess of an alkylene oxide, alkylated phenols, which have been treated with ethylene oxide (see French patent specification No. 823,454), condensation products of higher fatty acids with amino acids (see German patent specification No. 653,522) and the like. The said non-soapy synthetic emulsifiers are especially suitable when working with zirconium oxychloride, zirconium oxynitrate and the water soluble or dispersible hydrolysates obtainable therefrom. In this case, the water repellent effect is especially good when the quantity of the emulsifier is as small as possible, for instance, equal to about 1 g. per liter of the impregnating bath.

The impregnation of the material with the water-repellent organic substances and the zirconium compounds may be carried out in one or several baths. The dry or wet material can be treated, for instance, in a first bath with the zirconium compound and in a second bath with a paraffin emulsion. When using the above mentioned zirconium compounds which yield strongly acid solutions (i. e., zirconium oxychloride, zirconium oxynitrate and the water soluble or dispersible hydrolysates obtainable therefrom), the solutions or dispersions are buffered to a pH of about 3.8 to 4.2, for instance, by adding soda, sodium acetate, sodium tetraborate, etc. Similar effects are obtained, if the material, before or after impregnation with one of the said particular zirconium compounds, is treated with a neutralizing agent like, for instance, soda, sodium acetate, sodium tetraborate or the like. On the other hand, as above suggested, the paraffin, wax, or the like emulsion may be added to the zirconium bath. Particular good results with such impregnating baths are obtained when using zirconium oxychloride, zirconium oxynitrate and the water soluble or dispersible hydrolysates obtainable therefrom, and one of the above mentioned highly active synthetic emulsifiers. It is understood that other finishing compounds may be present in the bath like, for instance, colophony, synthetic resins and the like.

After impregnation with the said components the material is preferably squeezed or centrifuged and partly or entirely dried. Thereupon it is subjected to a treatment with alkalies and/or water

which is an important step in the process of the present invention. It is the purpose of this treatment to remove all hydrophilic substances like, for instance, water soluble electrolytes, soap or other emulsifiers from the material as far as possible. An alkaline treatment will give the desired improved results in all cases, i. e., with every kind of emulsion and zirconium compound. It is carried out by treating the material preferably at elevated temperature with aqueous solutions of the alkalies (caustic soda, sodium carbonate, ammonia, etc.), of alkaline reacting substances like sodium tetraborate, alkali salts of weak organic acids like the sodium salt of acetic acid, methylamino ethane sulfonic acid or methylamino acetic acid, and the like. It is sufficient when by this alkaline treatment the material is thoroughly wetted. Moreover, it is advantageous that the concentration of alkali is not too high. To the alkaline bath there may further be added small quantities of such wetting agents which can easily be removed by rinsing with water. For instance, solutions are used which contain per liter water 3 gs. soda or 2.5 gs. ammonia and 0.1 g. of the sodium salt of isobutyl naphthalene sulfonic acid. After the alkaline treatment the material is rinsed with water in order to remove the hydrophilic substances as far as possible from the material. It may be mentioned at this point that it is advantageous that from the beginning the quantity of electrolytes and other hydrophilic substances which are brought on the material is not too high so that they can more easily be removed from the material and will not impair the water repellent effect of the process. Finally, the material is again dried, which may be effected, for instance, by simply ironing.

In another modification of our invention, the alkali treatment of the impregnated material may be dispensed with, viz., if the material has been impregnated with a paraffin, wax, etc., emulsion which is free from soap and with a zirconium compound of the group of zirconium oxychloride, zirconium oxynitrate and the water soluble or dispersible hydrolysates obtainable therefrom. In this case it will be sufficient if the impregnated material is rinsed with water, preferably at elevated temperatures. The effect is improved if the material has been partially or totally dried between impregnating and rinsing it.

By following the indications given in the present specification it is possible to render all kind of textile material (for instance, cotton, artificial silk and staple fiber from viscose, cuprammonium cellulose and cellulose acetate solutions, wool, silk, mixed material from the afore-mentioned textile fibers, etc.) excellently and permanently water repellent. The results are especially improved in comparison with materials which have not been subjected to the after-treatment with alkalies and/or water, for instance, such as have been obtained according to the processes described in our co-pending application Ser. No. 221,452. The water repellent effect is so good that the treated materials in many cases show the so-called "pearl-off"-effect, i. e., water which is sprayed on fabrics impregnated according to the present process will immediately pearl off, leaving hardly any traces on the material. The water repellent finishes are, moreover, of excellent fastness to wet treatments, for instance, against washing. In most cases, the effect will withstand 5 or more washings with soap or soda without being appreciably impaired. The effect

is, moreover, resistant to decatizing and fulling.

It may be helpful to add a short description of the method according to which the water repellent effects obtainable according to the present process can be quantitatively measured. The fabric to be tested is sprayed with 1.51 of water of 25° C. from a height of 70 cms. at a pressure of 100 mm. Hg. The difference in weight of the fabric before and after spraying is measured and calculated in per cent of the original weight. The smaller the increase in weight, the better, apparently, is the water repellent effect.

The process of our invention is more fully illustrated by the following examples without, however, being limited thereto.

#### Example 1

A light thin fabric of viscose staple fiber is impregnated with an aqueous emulsion containing

|                              | Grams per 1 liter |
|------------------------------|-------------------|
| Paraffin and wax             | 8                 |
| Soap                         | 4                 |
| Zirconium acetate or formate | 25                |

After drying at 90° C., the fabric is subjected for 10 minutes at 80° C. to an alkaline treatment by means of an aqueous solution of 3 gs./l. sodium carbonate, whereupon it is thoroughly rinsed with water and dried.

The absorption of water amounts to 33% after 1 washing and 47% after 5 washings; whereas it is 110% in the untreated tissue.

#### Example 2

A dyed mixed fabric consisting of cotton and viscose staple fiber is impregnated with an emulsion containing zirconium acetate as described in

Example 1. After drying at 85° C., the tissue is dipped for 10 seconds into a bath of 90° C. containing per liter 2.5 gs. ammonia and 0.1 g. of the sodium salt of oleyl methyl taurine. Thereupon it is well rinsed with water and dried.

The absorption of water amounts to 18% after 1 washing and 19% after 5 washings, against 75% shown by the untreated tissue.

#### Example 3

A staple fiber fabric according to Example 1, is treated with an emulsion containing paraffin, wax and soap having dissolved therein 24 gs. of zirconium oxychloride (46% ZrO<sub>2</sub> content) per liter. Thereupon it is squeezed and the fabric is quickly passed through a 0.6% sodium acetate bath. After squeezing the tissue is dried and after-treated as described in Example 1.

The absorption of water amounts to 34% after 1 washing and 38% after 5 washings.

#### Example 4

A dyed woolen fabric is impregnated with an emulsion of paraffin, wax and soap, containing 24 gs. zirconium oxychloride per 1 liter (46% ZrO<sub>2</sub>-content). Thereupon the material is centrifuged and dipped for a short time into a bath containing 10 gs./l. of crystallized sodium acetate. After squeezing and drying the impregnated fabric is dipped for 15 seconds into a bath of 45° C. containing 2.5 gs. ammonia and 0.1 g. of the sodium salt of oleylmethyl taurine per 1 liter. After rinsing with water, drying at elevated tem-

perature and ironing of the still humid fabric, the water absorption amounts to 20% and 16% after 1 washing, 18% after 3 washings and 11% after 5 washings against 102% shown of the untreated fabric.

*Example 5*

A dyed mixed fabric from wool and viscose staple fiber (1:1) is treated with an emulsion thereof with 24 g./l. of zirconium oxychloride (46%  $ZrO_2$  content) and which has been brought to a pH of 4.2 by the addition of sodium carbonate and sodium acetate. After drying at 85° C., the fabric is dipped for 2 minutes into a bath of 40° C., containing 2.5 gs./l. of ammonia and 0.2 g./l. of the sodium salt of butyl naphthalene sulfonic acid. Thereupon the fabric is well rinsed with water and dried by ironing.

The absorption of water amounts to 8% after 1 washing and 12% after 5 washings.

*Example 6*

A mixed fabric from wool and viscose staple fiber according to Example 1, is impregnated with an emulsion of paraffin, wax and soap, containing 25 gs./l. zirconium oxynitrate which has been partially neutralized by means of 1.4 gs./l. sodium carbonate and 6 gs./l. crystallized sodium acetate. After squeezing and drying at 95° C., the fabric is treated for 5 minutes at 90° with a solution of 3 gs. sodium carbonate in 1 liter water. Thereupon the material is well rinsed with water and ironed.

The absorption of water amounts to 23% after 1 washing and 31% after 5 washings.

*Example 7*

When replacing in Example 6 zirconium oxynitrate by 24 gs./l. zirconium sulfate which has been neutralized by means of 10 gs./l. sodium carbonate and 4.8 gs./l. crystallized sodium acetate and working as described in the preceding example, the absorption of water amounts to 27% after one washing and to 38% after 5 washings.

When replacing zirconium oxynitrate by the equimolecular proportion of a zirconium hydroxide sol, which is, for instance, prepared by dialysis of a zirconium oxychloride solution and which can be employed without any neutralizing operation, the absorption of water amounts to 27% after 1 washing and 27% after 5 washings.

*Example 8*

A light thin mixed fabric consisting of wool and viscose staple fiber is impregnated as described in Example 3, and, after drying, is dipped into a bath containing, per liter water, 3 gs. sodium or ammonium bicarbonate, or 75 ccm. n/1 sodium lye or 2.5 gs. ammonia or 3 gs. sodium phosphate or 3 gs. borax or 5 gs. sodium stannate. Thereupon the fabric is well rinsed with water and dried. The absorption of water after several washings is similar to the values obtainable according to Example 3.

*Example 9*

A mixed fabric from wool and viscose staple fiber is impregnated with an emulsion consisting of paraffin, wax and soap, having incorporated therewith 24 gs. zirconium oxychloride and 12 gs.

borax per 1 liter. After squeezing and drying at 90° C., the fabric is treated for 5 minutes with a solution containing 3 gs. sodium carbonate per 1 liter water. Thereupon it is well rinsed with water and dried. The tissue thus obtained shows an especially soft touch which is not appreciably impaired on repeatedly washing.

The absorption of water amounts to 25% after 1 washing and 10 27% after 5 washings.

*Example 10*

Schappe silk is impregnated with an emulsion of paraffin, wax and glue, containing 24 gs./l zirconium oxychloride which has been partially neutralized with 18 gs./l. crystallized sodium acetate. The aftertreatment with ammonia and the further treatment is effected as described in Example 5.

20 The absorption of water amounts to 20% after 1 washing and 22% after 5 washings.

*Example 11*

25 A loosely woven mixed fabric consisting of wool and viscose cellulose staple fiber is impregnated with an emulsion containing per 1 liter 3 gs. paraffin, 2 gs. of a montanic acid ester, 2.5 gs. ammonium oleate and 24 gs. zirconium oxychloride (46%  $ZrO_2$  content) which has been partially neutralized by means of 18 gs. crystallized sodium acetate. After squeezing and drying in the heat, the fabric is wetted with a solution of 90° C. containing 3 gs. of sodium bicarbonate per 1 liter. Thereupon it is squeezed, well rinsed with water and dried at 90° C. The fabric thus impregnated shows good water repellent properties which are by no means impaired even after several washings.

*Example 12*

40 A mixed fabric consisting of wool and viscose staple fiber is impregnated with an emulsion containing per 1 liter water: 7.5 gs. triethanol amine-oleate, 3.2 gs. paraffin, 3.2 gs. ceresin, 2.8 gs. montanic acid ester, 24 gs. zirconium oxychloride (46%  $ZrO_2$ -content) and 0.44 g. aluminum (as hydroxide). Thereupon the fabric is squeezed and quickly passed through a 0.6% sodium acetate bath. After drying at 90° C., the fabric is treated for 2 minutes at 80–90° C. with a solution of 3 gs. soda+0.3 g. of the sodium salt of oleyl methyl taurine per 1 liter water, whereupon it is for several times rinsed with water and dried at elevated temperature.

The absorption of water amounts to 31% after 1 washing and 39% after 5 washings.

*Example 13*

60 A wet mixed fabric consisting of cotton and viscose staple fiber is treated on the jigger with an emulsion containing per 1 liter water 20 gs. of a weakly acid aqueous emulsion of paraffin (20%), glue (8%), aluminium hydroxide gel (6%), colophony (1%), 24 gs. zirconium oxychloride (46%  $ZrO_2$  content) and 4 gs. sodium acetate. Thereupon the fabric is passed through a 0.7% sodium acetate bath. After drying at about 90° C., the fabric is treated with a hot 0.3% sodium carbonate solution and then with a 0.1% warm soap solution and subsequently well rinsed with water. The fabric thus impregnated shows excellent water repellent properties.

*Example 14*

A fabric of viscose artificial silk having been pre-treated by means of a 0.2% soap solution and rinsed, is impregnated in the wet state with an emulsion as described in Example 13 having dissolved therein, in addition, 13.5 gs. borax. After having been squeezed and dried at 85° C., the fabric is treated for a short time with a 0.3% sodium carbonate solution at 90-95°, whereupon it is several times rinsed with water and dried by ironing.

The absorption of water amounts to  
32% after 1 washing and  
33% after 5 washings.

*Example 15*

The following impregnation bath is prepared: 62.5 gs. of an emulsion consisting of 8% paraffin, 8% ceresin, 7% artificial wax (montanic acid ester), 2% of an emulsifier (obtained by the condensation of oleyl alcohol with several mols ethylene oxide) and 75% water are pasted with 600 ccms. water of 70° C. This emulsion is added to a solution of 12 gs. zirconium oxychloride (46% ZrO<sub>2</sub>-content) in 300 ccms. water of 70° C. At 65° C. there are stirred into this bath 30 ccms. of a 10% aqueous sodium carbonate solution and, after cooling to 45° C., 2 ccms. glacial acetic acid and 1.2 gs. crystallized sodium acetate (20% aqueous solution). The bath shows then a pH of 3.9.

In this bath one of the following textile materials is treated at 45° C. for 1 minute: a loosely woven viscose staple fiber fabric, smooth undyed viscose artificial silk fabric, cellulose acetate artificial silk fabric, freshly precipitated deacidified loose cuprammonium cellulose staple fiber, dyed densely woven cotton popeline fabric (fabric for mackintoshes), thin loosely woven wool fabric, mixed fabric consisting of wool and viscose staple fiber (1:1) and a schappe silk fabric. Thereupon the materials are squeezed and dried in the usual manner. Before the first washing the materials are drawn for 1 minute through water of 95° C., whereby they are immediately wetted; they are then rinsed for a short time with water and dried in the drying-oven at 85-95° for 30 minutes. The materials thus impregnated show an excellent "pearl-off"-effect which is not impaired even after the fifth washing; they are, furthermore, fast to decatizing. The cuprammonium cellulose staple fiber is capable of being fulled for 32 hours without showing any decrease in its water-repellent capacity.

The treatment with hot water can also be carried out at lower temperatures, temperatures over 80° C., however, being preferred, since a more quickly wetting of the fabrics is effected thereby.

*Example 16*

The following impregnation bath is prepared: 75 gs. of an emulsion, containing 12% train oil ketone (obtainable by distillation of the calcium salts of the train oil fatty acids), 12% artificial wax (montanic acid ester), 0.3% soda, 1.4% of an emulsifier (obtainable by the condensation of oleyl alcohol with several mols ethylene oxide) and water are pasted with 250 ccms. water of 25° C. On the other hand, 12 gs. zirconium oxychloride (46% ZrO<sub>2</sub> content) are dissolved at 50° C. in 200 ccms water, whereto 30 ccms. 10% sodium carbonate solution and 2 ccms. glacial acetic acid are added. After cooling to 25°, the wax solution is stirred into the zirconium salt solution, whereupon ½ liter water and 7.5 ccms.

of a 20% aqueous solution of crystallized sodium acetate are added. The emulsion shows then a pH of about 3.9.

With this impregnating bath the fabrics mentioned in Example 15 are treated, the viscose staple fiber, artificial silk and cotton for 1 minute, the fabrics containing wool and silk only for 10 seconds. The fabrics are then squeezed and dried, with the exception of the silk, by exposing to the air for ½ hour. Thereupon the fabrics are dipped for 1 minute into hot water of 97°, shortly rinsed and dried in the drying oven at 85-95° for 30 minutes. In all cases, an excellent and permanent "pearl-off"-effect is reached, the fabrics showing, furthermore, a good fastness to decatizing. In the case of the viscose artificial silk it is advantageous to completely dry the fabric before subjecting it to the treatment with hot water; the water-repellent effect is still further improved thereby.

*Example 17*

An aqueous paraffin emulsion is prepared containing 10% paraffin, 10% ceresin, 8.75% artificial wax (montanic acid ester), 5% oleic acid, 0.7% sodium hydroxide and 1.25% of a condensation product of oleyl alcohol with several mols. ethylene oxide. 50 gs. of this emulsion are stirred into 350 ccms. water at 50° C. This solution is stirred at 45° C. into a solution of 12 gs. zirconium oxychloride (46% ZrO<sub>2</sub>-content) in 200 ccms. water, whereupon there are added 30 ccms. of a 10% aqueous sodium carbonate solution, 2 ccms. glacial acetic acid, 350 ccms. water of 25° C. and 1.2 gs. crystallized sodium acetate in form of a 20% aqueous solution. The impregnating bath thus prepared shows a pH of 3.9. The content of oleic acid imparts to the original paraffin emulsion a good stability and reduces the tendency of foaming of the bath.

In the bath thus prepared the textile fabrics mentioned in Example 15, are dipped for 1 minute at 40° C., whereupon they are squeezed, so that the viscose staple fiber fabric shows an increase in weight of 115% and then allowed to lay for ½ hour. The fabrics are then dipped into water of 95° C. for 1 minute, shortly rinsed with water and dried for 30 minutes in the drying oven at 85-95° C. All fabrics thus impregnated show an excellent and permanent water-repellent effect. The water-treatment can be carried out at 70° C. with a similar result.

*Example 18*

55 A dyed acetate artificial silk satin is impregnated with an emulsion containing per liter water 8 gs. paraffin and wax, 4 gs. soap and 24 gs. zirconium oxychloride and which is partly neutralized by addition of sodium acetate to a pH of 4.2.

56 The fabric is thereupon for a short time (15 sec.) immersed into an aqueous bath of 40° C. containing per liter 0.25 g. ammonia and 0.1 g. of the sodium salt of oleyl methyl taurin.

65 Thereafter the fabric is thoroughly rinsed with water and dried.

By this treatment the fabric has acquired water repellent properties of outstanding quality:

70 The absorption of water of the fabric before washing the same is 3%, and after five washings 5%, i. e., the fabric does not practically take up any water.

The "pearl-off" effect is excellent.

We claim:

1. Process for rendering textile material water

repellent which comprises impregnating the material with an emulsion containing paraffin, wax, a small quantity of a fatty acid, zirconium oxychloride and a condensation product of oleyl alcohol and of several molecular quantities of ethylene oxide serving as emulsifying agent, thereupon rinsing the material with hot water, whereby the hydrophilic substances are removed therefrom as far as possible, and finally drying the material at elevated temperature.

2. Process for rendering textile material water repellent which comprises impregnating the material with an emulsion being buffered with soda at a pH of 3.8-4.2 and containing paraffin, wax, a

small quantity of a fatty acid, zirconium oxychloride and a condensation product of oleyl alcohol and of several molecular quantities of ethylene oxide serving as emulsifying agent, thereupon rinsing the material with hot water, whereby the hydrophilic substances are removed therefrom as far as possible, and finally drying the material at elevated temperature.

3. A process as in claim 1 in which the textile material is cellulose acetate.

ARNOLD DOSER.

OTTO BAYER.

KARL HINTZMANN.